

## UNITED STATES PATENT OFFICE

2,599,093

## PIGMENTED CELLULOSE FIBER

William Lutton Craig, Westport, Conn., assignor  
to R. T. Vanderbilt Company, Inc., New York,  
N. Y., a corporation of New York

No Drawing. Application March 17, 1948.  
Serial No. 15,510

12 Claims. (Cl. 106—204)

1

This invention relates to new fibrous pigments or pigmented fibers or pulp and includes the new dry fibrous pigments and the process of producing them.

The new fibrous pigments or pigmented fibers are modified cellulosic pulp fibers containing precipitated within the fibers and on and around the fibers an amount of finely divided pigment, particularly calcium, barium or zinc pigments, e. g. calcium carbonate, barium or zinc sulfate or carbonate, etc. exceeding the dry weight of the fibers and advantageously in amount greatly exceeding the weight of fibers.

The new dry fibrous pigments or pigmented fibers are made by precipitating in and on and around the modified cellulosic fibers an insoluble pigment, with a considerable part of the precipitated pigment within the fibers. The new pigmented fibers are made by first subjecting the fibers in the form of a pulp to the action of a solution of calcium chloride, barium chloride or zinc chloride, containing an amount of chloride far exceeding the dry weight of the fiber, to effect swelling and hydration and modification and gelatinization of the fibers so that a large amount of chloride will be contained within the gelatinized fibers, and then precipitating the insoluble calcium, barium or zinc pigment by adding a solution of a soluble salt such as sodium carbonate or sulfate, aluminum sulfate, etc., to the fibers so treated with the chloride; followed by removal of the salt formed as a byproduct and drying the product under regulated conditions to give the dry pigmented fibers or fibrous pigment.

The present invention is based upon the discovery that cellulosic fiber stock (chemical, semi-chemical, or mechanical pulp) used in making paper, including cellulose fibers (chemical pulp) such as kraft, sulfite, soda pulp, etc. and groundwood (ligno-cellulose) fibers (mechanical pulp) can be treated with a solution of calcium, barium or zinc chloride to hydrate, modify and gelatinize the pulp fibers, and that the so modified cellulosic fibers can then be treated with a solution of a soluble salt such as sodium carbonate, sodium sulfate, etc. to precipitate an insoluble pigment such as calcium carbonate, barium sulfate, zinc sulfate or silicate or hydroxide largely within the modified fibers, as well as on and around the modified fibers; and that the resulting modified and pigmented stock, containing the pigmented modified fibers, can be freed from salt formed as a byproduct and dried under regulated conditions to give a valuable dry, fibrous pigment product, or pigmented fiber product, which can be stored and shipped

2

in a dry state and which can be readily reconverted into a fibrous pulp and used for admixture with other fibers for paper manufacture.

In my prior applications Serial Nos. 664,425, filed April 23, 1946, and 666,199, filed April 30, 1946, I have described the production of a new pigmented fiber stock in the form of a pulp by the treatment of cellulosic fibers with a strong solution of calcium chloride to effect modification of the fibers followed by treatment with, e. g., sodium carbonate to precipitate calcium carbonate in and on and around the fibers; and the use of such pigmented fiber stock for admixture with untreated fibers in making paper or for use in the outer layer in making laminated stock or both. According to the present invention, such pigmented fiber stock is freed from the greater part of its water and converted into a dry fibrous pigment or pigmented fiber which can be stored and shipped in a dry state and which can be readily reconverted into a fibrous pulp and used as a fibrous pigment for admixture with paper stock for paper manufacture.

The fibers which are used in making the new fibrous pigment include paper pulp fibers and particularly cellulosic fibers, including both chemical and semi-chemical pulp and groundwood fibers such as sulfite pulp, sulfate pulp, soda pulp, semi-chemical pulp, mechanical pulp, etc. The stock treated may be bleached or unbleached stock and may be stock which has been previously refined in a beater or refining engine or which may be unrefined stock, or which may be subjected to beating or refining in connection with the treatment of the pulp to produce the new fibrous pigment.

The pulp fibers are advantageously first treated with a strong solution of calcium chloride, containing an amount of calcium chloride much greater than the weight of the fibers, advantageously many times the amount of fibers (dry basis), in the pulp, and with the use of a sufficiently strong solution, or with beating of the pulp with a more dilute solution, to effect hydration and swelling and gelatinization and modification of the pulp fibers, so that a large part of the calcium chloride will be contained within the swollen hydrated fibers; after which the modified pulp is treated with a solution of a soluble salt which will precipitate an insoluble calcium compound as a pigment within as well as on and around the modified pulp fibers. A solution of sodium carbonate is advantageously used to give calcium carbonate as the pigment so precipitated in an exceedingly fine state of subdivision within and on and around the pulp fibers.

When the fibers are treated in the form of a pulp, e. g., 1% or 2% fibrous content (dry basis) or when a more concentrated stock is used, e. g., around 4% or 5% or 6% of fibers (dry basis) the calcium chloride is advantageously added in the form of dry calcium chloride and in amount two or more times the weight of the fibrous stock (dry basis). Thus with stocks containing around 4 or 5 or 6% of fibers (dry basis) the amount of calcium chloride is advantageously such as to form a solution of e. g. 13% or higher or up to 15 to 20% or more, and saturated calcium chloride solutions can be used. With more dilute pulps containing e. g., around 1% or 2% of fibers (dry basis) a more dilute calcium chloride solution can be used, e. g., a solution containing 5% or more calcium chloride or more advantageously a solution containing around 10% or more calcium chloride, with prolonged mechanical treatment or beating to effect swelling hydration, and gelatinization of the pulp fibers.

With strong calcium chloride solutions, e. g., around 13 to 20%, a profound modification of the cellulosic fibers takes place in a short period of time, e. g., 5 to 10 or 15 minutes, with proper agitation. The fibers become more or less gelatinous and transparent in appearance. With more dilute calcium chloride solutions prolonged beating of the pulp in a beater is advantageous to promote the hydrating and gelatinizing action and also to convert the pulp into a refined pulp.

Instead of adding dry calcium chloride to an ordinary pulp containing a small percentage of fibers, the treatment can be carried out by adding dry pulp stock (chemical, semi-chemical or mechanical pulp) to a more dilute aqueous solution of calcium chloride, advantageously a 10% solution, and with beating or refining of the pulp to promote the action of the calcium chloride on the fibers and to bring about the swelling and hydrating and gelatinizing action with resulting incorporation of a considerable amount of the calcium chloride within the fibers as well as on and around them. This method of treating dry pulp with an aqueous solution of calcium chloride is more fully described in my companion application Serial No. 15,509, now Patent No. 2,583,548 issued January 29, 1952.

After such treatment of the pulp fibers with calcium chloride the stock is treated with a solution of a soluble salt such as sodium carbonate (soda ash) or sodium borate, e. g., in the form of a 10% solution in sufficient amount to react with the calcium chloride and precipitate an insoluble pigment (e. g., calcium carbonate or calcium borate) in and on and around the modified fibers. The amount of added soluble salt is equal to or somewhat more or less than the amount which is sufficient to react with all of the calcium chloride used. With cellulose fibers (chemical pulp) the amount of soluble salt is advantageously slightly in excess of that required to react with all of the calcium chloride, but with groundwood fibers care should in general be taken to avoid any excess of the alkali salt which would darken or otherwise affect the stock, and with such stock the calcium chloride and sodium carbonate are used in exact reacting proportions or with a slight excess of calcium chloride.

The resulting treated and pigmented stock is highly hydrated and in general has much less strength than the untreated stock but it carries

the precipitated pigment distributed throughout the hydrated stock while pigment is also precipitated on the hydrated stock and in the water in which the stock is suspended.

This specially treated and modified stock is highly pigmented. The amount of pigment is in excess of the weight of the stock treated (dry basis) and particularly advantageous products are made by incorporating an amount of pigment which is twice the weight of the fibers or three times the weight of the fibers or even four or five times the weight of the fibers or more, as illustrated, for example, in Example 1, where the weight of the pigment is about 7.7 times the weight of the fibers, and in Example 2, where the weight of the pigments is about sixteen times the weight of the fibers.

The stock after treatment with the calcium chloride and with the soluble sodium salt will contain sodium chloride in solution. A large part of this salt will be removed when the fibrous stock is filtered or the main part of the water is separated from it but it is advantageous to wash the treated stock to effect more or less complete removal of the sodium chloride or the greater part of it before the pigmented stock is dried. The washing of the treated stock can be carried out by decantation or by washing in pulp washers with replacement of the sodium chloride solution with fresh water, care being taken that the water drawn off is clear or relatively clear water to avoid or minimize loss of finely suspended pigment during the washing operation.

This washed stock will contain the pigmented fibers or fibrous pigment with a relatively large amount of water. To produce the dry fibrous pigment or pigmented fibers this stock is freed from the main portion of its water by filtering or passing over a screen and advantageously in the form of a continuous sheet from which most of the water is drained or sucked by vacuum or by passing through pressure rolls to squeeze out as much water as possible. And the resulting wet pulp is then dried under regulated conditions to form the dry product.

It is important, for producing products which can be readily rehydrated and reconverted into pulp form with water, to avoid excessive drying and the production of a bone dry product, which is less valuable as a fibrous pigment. The drying can, however, be carried out rapidly by passing wet pigmented fibers through a continuous drier in sheet form and drying to the point where it still contains a small amount of water, e. g., around 5 to 10% more or less based on the fibrous content of the pigmented fibers. The product can also be air-dried but this will ordinarily take too long a time for practical operations. Ordinary drying rolls can be used with a limited time of contact of the continuous pigmented fiber sheet with the hot rolls to avoid excessive heating and drying. The wet fibrous pigment or pigmented fibers can also be broken up into lumps or into small pieces before drying. The dried product can also be broken up into lumps or pieces or into coarse powder form or the dried product can be formed into rolls or into laps for storage and shipment.

This new dry fibrous pigment or pigmented fibrous product will contain the finely divided precipitated pigment in amount exceeding the weight of the fibers treated and advantageously in amount two or three or four times the weight of the fibers or even more.

This new fibrous pigment is a valuable pigment

for use in paper making for admixture with paper pulp. If the cellulosic fibers treated are beaten or refined prior to or during the treatment the resulting fibrous pigment is a refined pulp stock which can be added to the furnish to be used for paper making after it has been prepared, e. g., by admixing it in regulated amounts, after rehydration, with the furnish before it goes to the paper machine. It can also advantageously be added to the beater and subjected to further refining or to the beater near the end of the refining treatment. It can be first rehydrated by admixing it with water and forming it into a pigmented fibrous pulp and added in this form to the pulp to be used for paper making.

The new fibrous pigment has an important advantage over ordinary pigments which are admixed with paper pulp in that a much larger proportion of the pigment is retained, and losses of pigment are minimized.

The invention will be further illustrated by the following specific examples but it will be understood that the invention is not limited thereto. The parts are by weight.

**Example 1.**—A groundwood stock of 3% consistency is prepared in a beater and to 333 parts of this stock containing 10 parts (dry basis) of fibers is added 99 parts of dry calcium chloride, with agitation. This calcium chloride dissolves and forms a strong solution which reacts with the groundwood stock. After about 15 to 30 minutes the stock is modified and hydrated and more or less gelled and 95 parts of sodium carbonate (soda ash) are then added in the form of a 10% solution. The sodium carbonate reacts rapidly with the calcium chloride that is in and on and around the fibers and a sufficient period of time, e. g., from 10 to 15 minutes is allowed to secure full precipitation. The precipitated fibrous pigment is then thoroughly washed to remove the salt (sodium chloride) that has been formed from the reaction. The washed pigment is then dried to a moisture content of around 5 to 10% either by drying in sheet form or by grinding or breaking up into smaller pieces before drying.

In the above example, about 77 parts of calcium carbonate are produced from 99 parts of dry calcium chloride, so that the amount of pigment is approximately 7.7 times the weight of the dry fibers.

**Example 2.**—An alpha-cellulose pulp is prepared by beating in the beater at a 3½% consistency and to 430 parts of the resulting stock containing 15 parts of alpha-cellulose (dry basis) is added 315 parts of dry calcium chloride, with continued stirring or agitation in the beater as described in Example 1, and then 304 parts of sodium carbonate (soda ash) are added in the form of a 10% solution and the process is continued as in Example 1.

The products of the above examples contain many times as much pigment as fiber (dry basis). With refined fibers the fibers may have a fluffy appearance on grinding. Although the dry product is made up mainly of pigment it is nevertheless fibrous in character, retaining in general the fibrous structure of the treated fibers but containing a large amount of precipitated pigment within and on and around the fibers. Thus in Example 2, about 244 parts of calcium carbonate will be produced from 315 parts of dry calcium chloride, so that the carbonate pigment is about 16 times the weight of the dry pulp (15 parts).

**Example 3.**—50 parts of groundwood pulp containing 3.5% of fibers (dry basis) are treated by

the addition thereto of 22 parts of anhydrous calcium chloride which is added in a solid state and dissolved in the water of the pulp and allowed to act thereon, e. g., about 10 minutes, with resulting modification of the pulp, the stock being stirred to insure thorough distribution of the calcium chloride and its action on the fibers. After the calcium chloride treatment there is added 20 parts of sodium carbonate (soda ash) dissolved in water to form a 10% solution and this solution is thoroughly admixed with the treated stock to bring about reaction between the sodium carbonate and the calcium chloride to precipitate calcium carbonate within the fibers of the treated stock as well as on and around the fibers of the stock. This reaction takes place in the period of about 5 to 10 minutes with continued agitation, but the action can be permitted to take place for a longer period of time. The sodium chloride solution is then removed from the stock and the stock is washed and then dried, e. g., in sheet form, to a product containing around 5 to 10% of water based on the fiber content of the fibrous pigment.

**Example 4.**—2400 parts of groundwood pulp of 2.5% fiber content equivalent to 60 parts of dry fibers are pumped to a treating tank and 440 parts of calcium chloride (74%  $\text{CaCl}_2$ ) are added and mixed thoroughly and dissolved and the agitation is continued for about 10 minutes to effect thorough treatment and gelling of the stock by the action of calcium chloride. A sodium carbonate solution is made by dissolving 300 pounds of soda ash in water to form a solution of about 10%. This solution is pumped into the calcium chloride treated stock and allowed to mix therewith, with continued agitation, until complete precipitation has occurred. The resulting treated stock in the form of a fibrous precipitate is pumped to storage tanks and allowed to settle without agitation. After settling, the top liquor (sodium chloride solution) is drawn off and replaced with fresh water to give a treated stock from which most of the water is removed, e. g., by passing onto a screen through which the water is largely removed and by passing the resulting sheet of wet fibrous pigment through a continuous drier for a sufficient time to dry the product to around e. g. 5 to 10% moisture content based on the fiber content of the fibrous pigment.

**Example 5.**—Bleached sulfite pulp in the form of ordinary sheets or laps is added to a 10% calcium chloride solution in a beater in amount sufficient to form a 2% stock (2% pulp dry basis) and the stock is subjected to a beating and refining treatment until the fibers become hydrated and swollen and somewhat gelatinous in character with little free water apparent around the swollen fibers and with resulting refining of the pulp to a greater or less extent. To the resulting mixture is added a 10% sodium carbonate solution containing an amount of sodium carbonate equivalent to the calcium chloride contained in the treated stock and the agitation or beating is continued for a period of e. g. 10 or 15 minutes to effect reaction of the sodium carbonate with the calcium chloride and the formation of calcium carbonate in and on and around the modified fibers. Sodium chloride is removed from the resulting stock by filtering or washing until the sodium chloride has been reduced, e. g., to below 0.01% sodium chloride on the solid content of the pulp. The resulting stock is then freed from water and dried to give a dry pigmented fiber. The resulting dry fibrous pigment

contained around 80% of calcium carbonate or an amount approximately four times the weight of the cellulose fibers (dry basis) and around 1 to 1½% of water, corresponding to around 5 to 7% of water on the fiber content of the fibrous pigment.

In the above examples the fibrous pigments contain a relatively small percentage of fiber and an amount of fine precipitated pigment several times the weight of the fiber. Such products are valuable fibrous pigments which can be admixed with water and reconverted into the form of a fibrous pigment stock or pulp. Although the fibrous content is relatively small, it nevertheless has a profound modifying effect in holding the finely divided precipitated calcium carbonate in a condition which minimizes loss of pigment and enables the pigment to be readily incorporated with ordinary paper pulp stock.

While it is possible by using a stock of higher concentration of fibers and a less excess of calcium chloride to produce pigmented fibers which contain approximately equal parts by weight of fiber and pigment, it is more advantageous to produce more highly pigmented fibers which contain at least twice as much pigment as fiber and even more advantageous for many purposes to produce pigmented fibers containing three or four or five times as much pigment as fiber or even higher percentages.

The new fibrous pigments or pigmented fibers can similarly be made with barium and zinc pigments, by the addition of dry pulp to a solution of barium chloride and zinc chloride or by adding dry barium chloride or dry zinc chloride to an aqueous pulp with mechanical treatment when required to effect swelling and hydrating and gelatinizing of the pulp fibers in the barium chloride or in the zinc chloride solution followed by precipitation of the insoluble barium or zinc pigment by the addition of a soluble salt such as sodium sulfate or alum (aluminum sulfate) or other soluble sulfate, or by adding sodium carbonate or other soluble carbonate, etc. to precipitate insoluble barium sulfate or zinc sulfate or a mixture of barium sulfate and aluminum hydrate or barium or zinc carbonate or zinc silicate or zinc hydroxide, etc. largely within and also on and around the cellulosic fibers.

The process in which barium chloride or zinc chloride is used is carried out as hereinbefore described in connection with calcium chloride by adding dry barium chloride or dry zinc chloride to a fibrous pulp or by adding dry pulp to the barium chloride or zinc chloride solution with mechanical treatment when needed to effect the hydrating and swelling and gelatinizing of the fibers so that a minimum of free water is present around the gelatinized fibers and by then precipitating the insoluble barium or zinc pigment by adding the soluble precipitating salt to the gelatinized stock.

The amount of insoluble barium or zinc pigment, as well as the amount of insoluble calcium pigment, will exceed the dry weight of the fibers and will advantageously be two or three or four or more times the weight of the fibers and the pigments will be largely contained in a fine precipitated state within the fibers as well as on and around the fibers.

The highly pigmented fibers containing the insoluble barium or zinc pigments when produced in pulp form can be dried under regulated conditions to give dry fibrous pigments which can be shipped and stored and used by admixing with

water to form a pulp which can then be used for admixture with untreated pulp or paper stock to give a pigmented paper stock and paper.

Such highly pigmented fibers containing barium or zinc pigments, after drying and converting into pulp form, as well as before drying and while in a pulp form, can be used for admixture with ordinary paper stock to supply fibrous pigment thereto as described in connection with the fibrous pigments containing insoluble calcium pigments in my prior applications Serial Nos. 664,425 and 666,199.

I claim:

1. Highly pigmented cellulosic pulp comprising the dried residue of swollen, hydrated and gelatinized cellulosic fibers and an amount of finely-divided pigment in excess of the dry weight of the fibers, and not exceeding about 16 times the weight of the fibers, the pigment being selected from the class which consists of precipitated inorganic salts of calcium, barium and zinc, the finely-divided pigment being largely within the cellulosic fibers but also on and around said fibers, the finely-divided pigment within the fibers having been precipitated in situ therein by reaction of one soluble salt with a second soluble salt while the second soluble salt is within the fibers while they are in a swollen, hydrated and gelatinized state, said pigment material forming a pulp-like mass on admixture with water.
2. Fibrous pigments such as defined in claim 1 in which the cellulosic fibers are chemical cellulose pulp fibers.
3. Fibrous pigments such as defined in claim 1 in which the fibers are groundwood fibers.
4. Fibrous pigments such as defined in claim 1 in which the pigment is more than twice the weight of the fibers.
5. Fibrous pigments such as defined in claim 1 in which the pigment is more than three times the weight of the fibers.
6. Fibrous pigments such as defined in claim 1 in which the pigment is more than four times the weight of the fibers.
7. Fibrous pigments such as defined in claim 1 in which the pigment is a calcium carbonate pigment precipitated by the reaction of calcium chloride and sodium carbonate.
8. Fibrous pigments such as defined in claim 1 in which the pigment is a calcium carbonate pigment precipitated by the reaction of calcium chloride and sodium carbonate, in amount more than twice the weight of the fibers.
9. Fibrous pigments such as defined in claim 1 in which the pigment is a calcium carbonate pigment precipitated by the reaction of calcium chloride and sodium carbonate, in amount more than three times the weight of the fibers.
10. Fibrous pigments such as defined in claim 1 in which the pigment is a calcium carbonate pigment precipitated by the reaction of calcium chloride and sodium carbonate, in amount more than four times the weight of the fibers.
11. Fibrous pigments such as defined in claim 1 in which the pigment is a precipitated barium compound pigment.
12. Fibrous pigments such as defined in claim 1 in which the pigment is a precipitated zinc compound pigment.

WILLIAM LUTTON CRAIG.

(References on following page)

## REFERENCES CITED

The following references are of record in the file of this patent:

## UNITED STATES PATENTS

| Number    | Name        | Date           | Number    |
|-----------|-------------|----------------|-----------|
| 348,958   | Flegle      | Sept. 14, 1886 | 404       |
| 354,477   | Just et al. | Dec. 14, 1886  | 262       |
| 2,080,437 | Rafton      | May 18, 1937   | 5 151,381 |
| 2,189,832 | Rafton      | Feb. 13, 1940  | 10        |

## FOREIGN PATENTS

| Country       | Date           |
|---------------|----------------|
| Great Britain | of 1869        |
| Great Britain | of 1873        |
| Great Britain | Sept. 27, 1920 |

## OTHER REFERENCES

Lottermoser et al., Kolloid-Zeitschrift, vol. 57, 1931, pgs. 206-208, 211-212, 216 and 221.  
 "An Introduction to the Chemistry of Cellulose," Marsh & Wood, 1938, pgs. 73, 77-78.